

## UNITED STATES PATENT OFFICE

ARTHUR J. WEINIG AND ROBERT E. CUTHEBERTSON, OF GOLDEN, COLORADO, ASSIGNEES  
TO THE AMERICAN METAL COMPANY, LIMITED, OF NEW YORK, N. Y., A CORPORA-  
TION OF NEW YORK

## ORE SEPARATION

No Drawing.

Application filed December 8, 1927. Serial No. 238,717.

This invention relates to ore separation, and more particularly to selective separation by flotation. The invention is particularly adaptable to the separation of ores comprising readily floatable gangue minerals, such as micaceous gangues and/or talcy gangues.

The term "ore" is to be understood as including concentrates, slimes, tailings or other products containing mixed minerals.

An object of this invention is to provide for the selective flotation in a more efficient and economical manner than has heretofore been practicable; and more particularly for the separation by flotation of respective metallic constituents of ore from the accompanying gangue and/or from each other.

The invention consists in treating the ore pulp prior to flotation with glue and alum, or with glue or alum alone, to thereby retard or inhibit the flotation of one or more of the minerals to be concentrated and/or the readily floatable gangue minerals; thereby effecting in an economical and more efficient manner separation of one or more constituent mineral elements from the accompanying gangue minerals.

We have discovered that glue, preferably in the form of a water solution or emulsion, has a selective depressant effect upon various minerals and upon all gangues, making its use valuable in selective flotation. One form of glue, which has been tried, and which is now being satisfactorily used, is a vegetable glue—a cereal derivative—the trade name of which is "Ceraline". It is to be understood, however, that the invention is not limited to the use of this class or particular kind of glue. For example, by adding glue to the ore pulp prior to flotation, it will so alter or inhibit the readily floatable gangue minerals, such for example as micaceous and talcy gangues, that they will be depressed during flotation into the tailing or reject, and thus permit the recovery of flotation concentrates of some of the valuable minerals free from contamination of the valueless gangue minerals. And we have further discovered that certain minerals when treated with glue are differentially in-

hibited retarded in flotation in increasing degrees respectively substantially in the following named order, and approximately to the relative degree indicated; the respective minerals being depressed accordingly. 55 While this is not a complete list of all minerals affected, it will serve as an illustration in connection with one successful embodiment of the invention as practiced in Pecos-Evangeline ore, and to be more particularly described following.

*Galena*.—Very little effect if the amount of glue used is kept within certain critical limits.

*Graphite*.—Depressed to some degree. 65

*Chalcopyrite*.—Depressing action of glue on chalcopyrite is noticeably stronger than on galena.

*Sphalerite*.—Depressing action of glue on resinous zinc sulfide is of very much the same 70 degree as its effect on chalcopyrite.

*Marmatite*.—The black zinc sulfides are noticeably depressed by glue.

*Pyrite*.—Pyrite is noticeably depressed by 75 the use of glue in approximately the same degree as marmatite.

*Molybdenite*.—Strongly depressed.

*Insoluble gangues*.—Glue exerts a strong depressing action on insoluble gangues in 80 general.

*Micaceous and talcy minerals*.—The micas and talcs are most strongly depressed of any of the above minerals.

The fact that glue, used within certain pre-determined limits has very little inhibiting action on galena, while acting as a strong depressant of micaceous and talcy gangue minerals, which ordinarily float even more readily than galena, makes it particularly 85 practicable to the application of lead cleaning of ores, such for example as Pecos ore or other complex ores; and the fact that glue acts as a noticeable depressant of marmatite, zinc and pyrite is of additional value. 95

We have also discovered that alum may be used as a depressing agent when added in small proportions, prior to flotation, to the ore pulp containing readily floatable gangue minerals, such for example as micaceous 100

and/or talcy gangue minerals, to so alter the flotation properties of the readily floatable gangue minerals that they will be depressed during flotation into the tailing or 5 reject and thus permit the recovery of flotation concentrates of the valuable minerals free from the contamination of the valueless gangue minerals. However, its present use for this purpose is not as practicable as the 10 use of glue to its present relatively greater cost.

We have further discovered that the use of alum as a floatable-gangue depressant in connection with a complex ore pulp containing 15 minerals such for example as lead, zinc and copper, possesses the added advantage of noticeably improving the flotation properties of certain minerals, such for example as copper, thereby causing said minerals to 20 float with the lead minerals, thus separating the copper from the zinc concentrate and insuring a higher recovery of the copper with the lead concentrate than could otherwise be obtained; a condition that is most 25 desirable for economical reasons.

The relative effect, and approximate degree of such effect, on various minerals such as are contained in the above types of ore, will be listed following for the purposes of 30 illustrating the present embodiment of the invention.

*Galena.*—Apparently unaffected by the use of alum.

*Chalcopyrite and copper minerals in general.*—Floatability of chalcopyrite and copper minerals in general is noticeably improved by the use of alum.

*Sphalerite and Marmatite.*—Alum appears to be a weak promoter for the zinc sulfides.

*Pyrite.*—Apparently unaffected.

*Insoluble gangues.*—Insoluble gangues in general are not visibly depressed.

*Micaceous and talcy minerals.*—Very noticeably depressed if alum is employed in sufficient quantity.

It will therefore be seen that with the use of alum in conjunction with glue, the alum activates the floatability of copper minerals, thereby counteracting and substantially neutralizing the depressing action of the glue on such minerals, and at the same time increasing the depressing action of gangues such for example as micaceous and talcy gangues.

Following these discoveries we have found that a judicious use of a combination of glue and alum may be employed to great advantage. For example, in the separation of complex ores such as Pecos ore, the depressing effect of glue upon chalcopyrite is of considerable disadvantage, and in such case the use of alum in addition to glue improves 65 the flotation of such minerals as chalcopy-

rite, while acting cumulatively with the glue to additionally depress certain other minerals such as micaceous and talcy gangues. In such case the glue is employed primarily for the elimination of micaceous and talcy gangue minerals, and incidentally for its inhibiting action on insoluble gangues in general, as well as on marmatite and pyrite. Alum is added in small quantity primarily to promote the flotation of chalcopyrite and thus overcome the detrimental effect of glue in depressing the copper to some extent, and also to exert additional depressing action on the talcy and micaceous minerals. 70 75

It is to be understood that the proportion of glue and/or alum to be used will depend upon certain variables, such for example as the quality and/or character of ore treated; and that the proper proportion may be ascertained by suitable tests, all of which will be understood by those skilled in the art 80 85 after understanding our invention.

The following examples will serve to illustrate the advantages of the invention; and show an embodiment of the invention as 90 practiced, for example on "Pecos-Evangeline ore". It is to be noted, however, that the method of procedure in the following Example No. 1 does not comprise the novel subject matter of this invention; this example being given merely as a means of comparison to illustrate the advantages of the invention over the method as heretofore practiced on ore of this character. 95

#### Example No. 1

In this example separation by froth flotation was practiced in a manner well known to those skilled in the art, to separate the lead and zinc froths; with the exception of the aeration conditioning treatment step which forms the subject matter of copending application Serial No. 233,876 filed October 4, 1927. 100 105

2520 grams of Pecos (Evangeline) ore, containing mixed lead, zinc, copper and iron sulfides, was ground to an 80 mesh fineness in a ball mill with water, conditioned for 90 minutes with aeration prior to lead flotation; this conditioning being for the purpose of inhibiting the flotation of the iron minerals; which conditioning by aeration per se forms no part of the present invention, being included in the subject matter of application 110 115 Serial No. 233,876 filed October 4, 1927. And the following reagents were then added in proportions enumerated:

|                                     | Pounds |
|-------------------------------------|--------|
| Sodium cyanide per ton ore-----     | 0.25   |
| Cresylic acid per ton ore-----      | 0.06   |
| Potassium xanthate per ton ore----- | 0.12   |

This charge was then placed in a flotation machine, and the machine started. The lead 120 130

froth was then removed; time of lead flotation 12 minutes. Then

0.06 lbs. pine oil per ton ore

0.2 lbs. xanthate per ton ore

5 2.5 lbs. copper sulphate per ton ore, and  
4.0 lbs. lime per ton ore

were added to the pulp remaining in the flotation machine and the zinc froth was then removed; time of zinc flotation 15 minutes. 10 The pulp dilution was approximately 4:1 and the temperature approximately 65° F.

The results of the run are shown following:

| Product      | Per cent of total | Assays |      |      |      | Per cent recovery |       |       |       |
|--------------|-------------------|--------|------|------|------|-------------------|-------|-------|-------|
|              |                   | % Pb   | % Cu | % Zn | % Fe | % Ins.            | of Pb | of Cu | of Zn |
| Heads.....   | 100               | 5.4    | 2.11 | 18.0 | 9.1  | 39.7              |       |       |       |
| Pb conc..... | 25.4              | 17.6   | 6.05 | 9.7  |      | 38.3              | 84    | 69    | 14    |
| Zn conc..... | 26.0              | 1.7    | 1.69 | 53.5 |      |                   | 2.5   | 3     | 20    |
| Tails.....   | 48.6              | 1.4    | .51  | 3.5  |      | 55.5              | 13    | 11    | 9     |
|              |                   |        |      |      |      |                   |       |       | .72   |

#### Example No. 2

23 In this example glue was used as inhibitor in separating the rougher lead froth, and in the lead cleaner flotation operation glue was also used, as will be more particularly pointed out in the following procedure.

33 2511 grams of Pecos (Evangeline) ore, containing mixed lead, zinc, copper and iron sulfides, was ground to an 80 mesh fineness in a ball mill with water and the following reagents added in proportions enumerated:

|                                        | Pounds |
|----------------------------------------|--------|
| Sodium cyanide per ton ore.....        | 0.25   |
| Animal glue per ton ore.....           | 0.9    |
| Cresylic acid per ton ore.....         | 0.06   |
| 40 Potassium xanthate per ton ore..... | 0.12   |

45 This charge was then placed in a flotation machine, and the machine started. The lead froth was then removed; time of lead flotation 12 minutes. Then

0.06 lbs. pine oil per ton ore

0.2 lbs. xanthate per ton ore

2.5 lbs. copper sulphate per ton ore, and

4.0 lbs. lime per ton ore

50 were added to the pulp remaining in the flotation machine and the zinc froth was then removed; time of zinc flotation 15 minutes: results as follows:

#### Example No. 2a

| Product            | Per cent of total | Assays |      |      |      | Per cent recovery |       |       |         |
|--------------------|-------------------|--------|------|------|------|-------------------|-------|-------|---------|
|                    |                   | % Pb   | % Cu | % Zn | % Fe | of Pb             | of Cu | of Zn | of Ins. |
| Headings.....      | 100               | 5.4    | 2.11 | 18.0 | 9.1  |                   |       |       |         |
| Crude Pb conc..... | 26.5              | 1.12   | 12.5 | 35.0 | 82   | 8                 | 12    | 14.30 |         |
| Zn conc.....       | 32.2              | 1.1    | 5.30 | 42.2 | 4.9  | 7                 | 76    | 78    | 3.09    |
| Tails.....         | 51.6              | 1.2    | 0.71 | 3.3  |      | 11                | 16    | 10    | 81.71   |

65 Then the lead froth was given a cleaner

flotation after the addition of 0.2 lbs. glue per ton ore and 0.04 lbs. cresylic acid per ton ore and the lead concentrate removed; time of lead cleaner flotation 5 minutes. The pulp dilution was approximately 4:1 and the 70 temperature approximately 65° F.

The results of the run are shown following:

#### Example No. 2b

| Product               | Per cent of total | Assays |      |      |        | Per cent recovery |       |       |         |
|-----------------------|-------------------|--------|------|------|--------|-------------------|-------|-------|---------|
|                       |                   | % Pb   | % Cu | % Zn | % Ins. | of Pb             | of Cu | of Zn | of Ins. |
| Pb conc.....          | 7.8               | 42.5   | 1.08 | 14.8 | 17.2   | 63                | 4     | 7     | 3.38    |
| Pb cleaner tails..... | 8.4               | 11.7   | 1.11 | 10.4 | 51.5   | 19                | 4     | 5     | 10.92   |

#### Example No. 3

This example illustrates a test run in which 85 alum was used as an inhibitor, and in which ore was conditioned by aeration for a period of 90 minutes prior to lead flotation; this conditioning being for the purpose of inhibiting the flotation of the iron minerals; 90 which conditioning by aeration per se forms no part of the present invention, being included in the subject matter of a separate application. The test procedure is given following.

2510 grams of Pecos (Evangeline) ore, containing mixed lead, zinc, copper and iron sulfides, were ground to an 80 mesh fineness in a ball mill with water and the following 95 reagents added in proportions enumerated:

|                                     | Pounds |
|-------------------------------------|--------|
| Sodium cyanide per ton ore.....     | 0.25   |
| Alum per ton ore.....               | 4.10   |
| Cresylic acid per ton ore.....      | 0.06   |
| Potassium xanthate per ton ore..... | 0.12   |

This charge was then placed in a flotation machine, and the machine started. The lead froth was then removed; time of lead flotation 12 minutes. Then

|                                           | Pounds |
|-------------------------------------------|--------|
| 0.06 lbs. pine oil per ton ore            |        |
| 0.2 lbs. xanthate per ton ore             |        |
| 2.5 lbs. copper sulphate per ton ore, and |        |
| 4.0 lbs. lime per ton ore                 |        |

were added to the pulp remaining in the flotation machine and the zinc froth was then removed; time of zinc flotation 15 minutes. The pulp dilution was approximately 4:1 and the temperature approximately 65° F.

The results of the run are shown following:

| Product       | Per cent of total | Assays |      |      |      | Percent recovery |       |       |         |
|---------------|-------------------|--------|------|------|------|------------------|-------|-------|---------|
|               |                   | % Pb   | % Cu | % Zn | % Fe | of Pb            | of Cu | of Zn | of Ins. |
| Headings..... | 100               | 5.4    | 2.11 | 18.0 | 9.1  | 39.7             |       |       |         |
| Pb conc.....  | 17.5              | 24.6   | 9.9  | 13.3 |      | 17.7             | 81    | 74    | 12      |
| Zn conc.....  | 29.6              | 1.9    | 1.38 | 50.2 |      | 5.7              | 10    | 17    | 80      |
| Tails.....    | 52.9              | 0.9    | 0.37 | 2.9  |      |                  | 9     | 9     | 8       |

120 125 130

## Example No. 4

This example illustrates a test run in which alum and glue were used in the lead cleaner operation only, and in other respects this test was conducted in general similarly to Example No. 3, as will be noted from the following test procedure:

250 grams of Pecos (Evangeline) ore containing mixed lead, zinc, copper and iron sulfides were ground to an 80 mesh fineness in a ball mill with water and conditioned by aeration for 90 minutes, and the following reagents added in proportions enumerated:

|                                | Pounds |
|--------------------------------|--------|
| Sodium cyanide per ton ore     | 0.25   |
| Cresylic acid per ton ore      | 0.06   |
| Potassium xanthate per ton ore | 0.12   |

This charge was then placed in a flotation machine, and the machine started. The lead froth was then removed; time of lead flotation 12 minutes. Then

0.06 lbs. pine oil per ton ore  
0.2 lbs. xanthate per ton ore  
2.5 lbs. copper sulphate per ton ore, and  
4.0 lbs. lime per ton ore

were added to the pulp remaining in the flotation machine and the zinc froth was then removed; time of zinc flotation 15 minutes.

## Example No. 4a

| Product  | Per cent of total | Assays      |             |             |               | Per cent recovery |       |       |         |
|----------|-------------------|-------------|-------------|-------------|---------------|-------------------|-------|-------|---------|
|          |                   | Per cent Pb | Per cent Cu | Per cent Zn | Per cent Ins. | of Pb             | of Cu | of Zn | of Ins. |
| Heads    | 100               | 5.4         | 2.11        | 18          | 39.7          |                   |       |       |         |
| Pb conc. | 26.4              | 17.2        | 6.98        | 9.72        | 38.0          | 84                | 69    | 14    | 26      |
| Zn conc. | 26.0              | 0.7         | 1.00        | 53.5        | 2.6           | 3                 | 20    | 77    | 2       |
| Tailings | 48.6              | 1.4         | .51         | 3.5         | 55.5          | 13                | 11    | 9     | 72      |

Then the lead froth was given a cleaner flotation after the addition of 0.3 lbs. glue per ton ore and 1.5 lbs. alum per ton ore and 0.04 lbs. cresylic acid per ton ore and the lead concentrate removed; time of lead cleaner flotation 5 minutes. The pulp dilution 50 was approximately 4:1, and the temperature approximately 65° F.

The results of the run are shown following:

## Example No. 4b

| Product          | Per cent of total | Assays      |             |             |               | Per cent recovery |       |       |         |
|------------------|-------------------|-------------|-------------|-------------|---------------|-------------------|-------|-------|---------|
|                  |                   | Per cent Pb | Per cent Cu | Per cent Zn | Per cent Ins. | of Pb             | of Cu | of Zn | of Ins. |
| Pb conc.         | 11.7              | 30.8        | 10.3        | 12.9        | 11.0          | 68                | 55    | 8     | 3       |
| Pb cleaner tails | 13.7              | 6.4         | 2.37        | 7.0         | 61.5          | 16                | 14    | 6     | 23      |

For purposes of comparing the relative

merits of the respective examples above given, a resumé of each of the above tests is given following in combined tabulated form.

## Tabulation crude Pb concentrates 70

| Test                    | Wt.  | Assays      |             |             |               | Per cent recovery |       |       |         |
|-------------------------|------|-------------|-------------|-------------|---------------|-------------------|-------|-------|---------|
|                         |      | Per cent Pb | Per cent Cu | Per cent Zn | Per cent Ins. | of Pb             | of Cu | of Zn | of Ins. |
| 1. Without glue or alum | 25.4 | 17.6        | 6.06        | 9.7         | 38.3          | 84                | 69    | 14    | 26      |
| 2. With glue            | 16.2 | 26.5        | 1.12        | 12.5        | 36.0          | 82                | 8     | 12    | 14.3    |
| 3. With alum            | 17.5 | 24.6        | 9.9         | 13.3        | 17.7          | 81                | 74    | 12    | 7.81    |

80

## Tabulation cleaned Pb concentrates

| Primary                  | Cleaning            | Wt.  | Assays      |             |             |               | Per cent recovery |       |       |         |
|--------------------------|---------------------|------|-------------|-------------|-------------|---------------|-------------------|-------|-------|---------|
|                          |                     |      | Per cent Pb | Per cent Cu | Per cent Zn | Per cent Ins. | of Pb             | of Cu | of Zn | of Ins. |
| 2. With glue             | Glue                | 7.8  | 42.5        | 1.08        | 14.8        | 17.2          | 63                | 4     | 7     | 3.38    |
| 1. Without glue and alum | Glue, glue and alum | 11.7 | 30.8        | 10.3        | 12.9        | 11.0          | 68                | 55    | 8     | 3.0     |

90

It will be seen from the composite table above that in Example No. 1 where no glue or alum were used a larger amount of copper and a greater proportion of zinc and a greater amount of insolubles were carried over with the lead concentrate than was the case in Example No. 2 where glue was used as inhibitor. It will be seen that in Test No. 3 where alum was used in place of glue a larger proportion of copper was carried over in the lead concentrate than in either the case without the use of glue or with the use of glue, and that the insolubles carried over were less than in either Tests 1 or 2. It will further be noted that in Test 4 where alum and glue were used, the insolubles were cut down from 3.38 to 3., being due to the additive inhibitory effect of the alum, and by the use of alum 55% of copper was carried over with the lead concentrate as against 8% with the use of glue only; thereby clearly illustrating the various advantages pointed out hereinbefore; and illustrating a greatly improved selectivity which is possible in lead flotation by the use of this invention.

Another important feature of the invention, which is illustrated in the table setting forth the differential inhibitory effect produced respectively on the various minerals of a complex ore by the use of glue, is that marmatite is noticeably depressed by the addition of glue prior to flotation; and this is of importance due to the fact that marmatite is comprised of a combination of zinc and iron sulfides, and it is particularly desirable to inhibit the flotation of the iron contained in the marmatite. And likewise, and for the same purpose, the depressing effect on

100

105

110

115

120

125

130

pyrite, by the use of glue, is highly advantageous.

Having thus described our invention with particularity with reference to the preferred method of carrying out the same, it will be obvious to those skilled in the art, after understanding our invention, that various changes and modifications may be made therein without departing from the spirit and scope of our invention, and we aim in the appended claims to cover such changes and modifications as are within the scope of the invention.

What we claim as new and desire to secure by Letters Patent is:

1. Method of separation by flotation of gangue from other minerals, which consists in adding to the ore pulp containing lead, copper and readily floatable gangue, prior to flotation and in addition to suitable flotation agencies a small proportion of the glue sufficient to inhibit the flotation of said copper and said readily floatable gangue.

2. Method of separation of ore containing lead, copper and readily floatable gangue material which consists in separating valuable lead minerals by the agency of suitable flotation agents while inhibiting the flotation of copper and relatively valueless gangues composed of materials other than metallic sulfide otherwise floatable, such as micaceous and talcy gangues, by addition to the ore pulp prior to flotation of a small proportion of glue to thereby depress said copper and gangue minerals.

3. Method of ore separation by froth flotation, which consists in selectively separating the gangue from other mineral constituents of said ore by the use of flotation agents while differentially reducing the flotation properties of some of said minerals by addition prior to flotation of a small proportion of glue to depress the gangue and also adding prior to flotation a small proportion of alum to thereby substantially neutralize the said reduction of the flotation property of at least one of said minerals other than the gangue.

4. Method of selective separation by froth flotation of complex ores containing lead, copper, and normally readily floatable gangue by the use of suitable flotation agencies, which comprises adding prior to flotation glue which acts as a strong depressant of said floatable gangues and also as a depressant of said copper and in such proportion as not to substantially affect the flotation properties of lead, and adding also prior to flotation a small proportion of alum which oppositely affects the flotation property of said copper substantially to the same degree and also acts as a further depressant of said gangues, while leaving substantially unaffected the flotation properties of said lead, whereby the flotation properties of said lead and copper are substantially unaffected and the inhibition to flotation of said gangues is greatly improved.

copper are substantially unaffected and the inhibition to flotation of said gangues is greatly improved.

5. Method of separating lead sulfide from an ore containing copper and normally readily floatable gangue composed of material other than metallic sulfide by froth flotation by the use of suitable flotation agencies, which comprises adding prior to flotation two agents which act cumulatively to inhibit the flotation of said copper and said gangue consisting of matter other than metallic sulfide while leaving substantially unaffected the flotation of said lead sulfide.

6. Method of separation by flotation of gangue from metallic sulfides, which consists in adding to the ore pulp containing copper and readily floatable gangue minerals belonging to the group of micaceous and talcy gangues prior to flotation and in addition to suitable flotation agencies a small proportion of glue sufficient to inhibit the flotation of said copper and said readily floatable gangues.

7. Method of separation by froth flotation of readily floatable gangue minerals from other valuable minerals, which consists in separating lead and copper constituents of said minerals by the use of flotation agents, one of which is glue, and each of said agents affecting differently the flotation properties of said lead and copper, and each of said agents acting cumulatively to depress the readily floatable gangue.

8. Method of selective separation by froth flotation of complex ores containing lead, copper, and normally readily floatable gangue by the use of suitable flotation agencies which comprises adding prior to flotation material which acts as a strong depressant of said floatable gangues and also a depressant of said copper and in such proportion as not to substantially affect the flotation properties of lead, and adding also prior to flotation a small proportion of material which oppositely affects the flotation property of said copper substantially to the same degree and also acts as a further depressant of said gangues, while leaving substantially unaffected the flotation properties of said lead, whereby the flotation properties of said lead and copper are substantially unaffected and the inhibition to flotation of said gangues is greatly improved.

9. A process of the kind described which comprises adding to the ore pulp containing lead and floatable talcy gangue in addition to suitable flotation material, a small proportion of materials selected from a group consisting of glue and alum, and floating the lead while depressing the talcy gangue.

10. A process of the kind described which comprises adding to ore pulp containing lead, iron sulfides and gangue material other than sulfide and in addition to suitable flotation

70

75

80

116

123

material, a small proportion of glue and floating the lead while depressing the iron and gangue.

In testimony whereof we have signed our names to this specification.

**ARTHUR J. WEINIG.  
ROBERT E. CUTHBERTSON.**

**CERTIFICATE OF CORRECTION.**

**Patent No. 1,906,029.**

**April 25, 1933.**

**ARTHUR J. WEINIG, ET AL.**

It is hereby certified that error appears in the printed specification of the above numbered patent requiring correction as follows: Page 1, line 40, for "fiotation" read "flotation", and line 51, before "retarded" insert the word "or"; page 2, line 10, after "glue" insert "due"; and lines 109 and 121, for the Serial No. "233,876" read "223,876"; page 4, line 60, in the boxed heading, column 4, for "Cn" read "Cu", and line 68, for "folowing" read "following"; and that the said Letters Patent should be read with these corrections therein that the same may conform to the record of the case in the Patent Office.

Signed and sealed this 13th day of June, A. D. 1933.

**M. J. Moore.**

**(Seal)**

**Acting Commissioner of Patents.**

material, a small proportion of glue and floating the lead while depressing the iron and gangue.

In testimony whereof we have signed our names to this specification.

**ARTHUR J. WEINIG.  
ROBERT E. CUTHBERTSON.**

**CERTIFICATE OF CORRECTION.**

**Patent No. 1,906,029.**

**April 25, 1933.**

**ARTHUR J. WEINIG, ET AL.**

It is hereby certified that error appears in the printed specification of the above numbered patent requiring correction as follows: Page 1, line 40, for "fiotation" read "flotation", and line 51, before "retarded" insert the word "or"; page 2, line 10, after "glue" insert "due"; and lines 109 and 121, for the Serial No. "233,876" read "223,876"; page 4, line 60, in the boxed heading, column 4, for "Cn" read "Cu", and line 68, for "folowing" read "following"; and that the said Letters Patent should be read with these corrections therein that the same may conform to the record of the case in the Patent Office.

Signed and sealed this 13th day of June, A. D. 1933.

**M. J. Moore.**

**(Seal)**

**Acting Commissioner of Patents.**

**CERTIFICATE OF CORRECTION.**

**Patent No. 1,906,029.**

**April 25, 1933.**

**ARTHUR J. WEINIG, ET AL.**

It is hereby certified that error appears in the printed specification of the above numbered patent requiring correction as follows: Page 1, line 40, for "fiotation" read "flotation", and line 51, before "retarded" insert the word "or"; page 2, line 10, after "glue" insert "due"; and lines 109 and 121, for the Serial No. "233,876" read "223,876"; page 4, line 60, in the boxed heading, column 4, for "Cn" read "Cu", and line 68, for "folowing" read "following"; and that the said Letters Patent should be read with these corrections therein that the same may conform to the record of the case in the Patent Office.

Signed and sealed this 13th day of June, A. D. 1933.

**M. J. Moore.**

**(Seal)**

**Acting Commissioner of Patents.**